

# UNITED STATES PATENT OFFICE.

JAMES HEBBARD AND RASMUS JOHN HARVEY, OF BROKEN HILL, NEW SOUTH WALES,  
AUSTRALIA, ASSIGNEES, BY MESNE ASSIGNMENTS, TO MINERALS SEPARATION  
NORTH AMERICAN CORPORATION.

## SEPARATION OF METALLIC SULFID ORES.

1,260,668.

Specification of Letters Patent.

Patented Mar. 26, 1918.

No Drawing.

Application filed August 28, 1914. Serial No. 653,737.

To all whom it may concern:

Be it known that we, JAMES HEBBARD and RASMUS JOHN HARVEY, subjects of the King of England, both residing at Central Mine, 5 Broken Hill, New South Wales, Australia, have invented certain new and useful Improvements in the Separation of Metallic Sulfid Ores, of which the following is a specification.

10 This invention relates to certain matters in the separation of mixed zinc and lead sulfid ores and refers more especially to the treatment of slimes.

In this specification the term "ores" is 15 intended to include concentrates, tailings, slimes, and other products containing mixed metallic sulfids.

The object of this invention is to provide an improved method of effecting a differential or preferential flotation separation of 20 lead sulfids (galena) from zinc sulfids (blende).

We have discovered that if mixed sulfid ores and more especially slimes are subjected 25 to froth flotation separation preferably with a small quantity of an emulsifying agent with agitation and aeration in an acid solution in which the quantity of acid is less than that required to produce a collective 30 float of both the lead and zinc sulfids a preferential flotation of the lead sulfids from the zinc sulfids can be effected. If the residues are then subjected to further flotation separation treatment with agitation and 35 aeration and in the same circuit liquors with the addition of a frothing agent such as eucalyptus oil float concentrates relatively rich in zinc can be obtained.

The acid (preferably sulfuric acid) which 40 is used in the first instance for the preferential flotation of the lead sulfids may be added to the circuit liquors or the ores may be submitted to a preliminary digestion in an acid solution in which case the acid solution 45 would be used in a preliminary mixing vessel. We have found that a better separation is effected if an emulsifying agent is present in the circuit liquors even if only in minute quantities. If circuit liquors previously used in froth flotation separation are employed (which are more or less air emulsified) then as a rule no addition of any emulsifying agent is required to float the lead sulfids. But if clean fresh water is

used then the addition of a small quantity of an emulsifying agent is advantageous.

The following is an example of an application of this invention:

A Broken Hill dump slime assaying 19% lead and 21% zinc was subjected to flotation separation in a circuit liquor which had previously been used in froth flotation separation, an amount of sulfuric acid equivalent to 22 lbs. per ton of ore treated being added with the feed. No addition of any frothing or emulsifying agent was made. The float concentrates produced from the first box assayed 66% lead and 9.8% zinc and averaging the float products from the twelve boxes in the series a ready concentrate assaying 70 50.5% lead and 21.2% zinc was obtained representing a recovery of 62.9% lead.

What we claim as our invention and desire to secure by Letters Patent is:

1. A process for the separation of lead sulfid from zinc sulfid in ores containing mixed lead and zinc sulfids which consists in submitting such an ore to treatment with an acid solution containing a mineral acid in quantity less than the normal quantity for froth flotation separation, and to agitation and aeration, so as to form a froth in which the lead sulfid predominates, and separating the froth.

2. A process for the separation of lead sulfid from zinc sulfid in ores containing mixed lead and zinc sulfids which consists in submitting such an ore to treatment with an acid solution containing a mineral acid in quantity less than the normal quantity for froth flotation separation, and to agitation and aeration, so as to form a froth in which the lead sulfid predominates, and thereafter submitting the tailings to a further froth flotation treatment with a frothing agent for the flotation of a froth in which the zinc sulfid predominates, and separating the froth.

3. A process for the separation of lead sulfid from zinc sulfid in ores containing mixed lead and zinc sulfids which consists in submitting such an ore to a flotation separation treatment by agitation and aeration in water containing a quantity of mineral acid less than is required to produce a collective float of both the lead and zinc sulfids and containing a frothing agent in less than the normal quantity for froth flotation.

tion separation, so as to form a froth in which the lead sulfid predominates, and separating the froth.

4. A process for the separation of lead sulfid from zinc sulfid in ores containing mixed lead and zinc sulfids which consists in submitting such an ore to a flotation separation treatment by agitation and aeration in water containing a quantity of mineral acid less than is required to produce a collective float of both the lead and zinc sulfids and containing a frothing agent in less than the normal quantity for froth flotation separation so as to form a froth in which the lead sulfid predominates, and thereafter submitting the tailings to a further froth flotation treatment with the addition of a frothing agent for the flotation of a froth in which the zinc sulfid predominates, and separating the froth.

5. A process for the separation of lead sulfid from zinc sulfid in ores containing mixed lead and zinc sulfids which consists in submitting such an ore to treatment with a solution containing sulfuric acid in quantity less than the normal quantity for froth flotation separation, and to agitation and aeration, so as to form a froth in which the lead sulfid predominates, and separating the froth.

6. A process for the separation of lead sulfid from zinc sulfid in ores containing mixed lead and zinc sulfids which consists in submitting such an ore to treatment with a solution containing sulfuric acid in quantity less than the normal quantity for froth flotation separation, and to agitation and aeration, so as to form a froth in which the lead sulfid predominates, and thereafter submitting the tailings to a further froth flotation treatment with the addition of a frothing agent for the flotation of a froth in which the zinc sulfid predominates, and separating the froth.

7. A process for the separation of lead sulfid from zinc sulfid in ores containing mixed lead and zinc sulfids which consists in submitting such an ore to a flotation separation treatment by agitation and aeration in water containing eucalyptus oil in less than the normal quantity for froth flotation separation, with the addition of a quantity of sulfuric acid less than is required to produce a collective float of both the lead and zinc sulfids, so as to form a froth in which the lead sulfid predominates, and separating the froth.

8. A process for the separation of lead sulfid from zinc sulfid in ores containing mixed lead and zinc sulfids which consists in submitting such an ore to a flotation separation treatment by agitation and aeration in water containing eucalyptus oil in less than the normal quantity for froth flotation, with the addition of a quantity of sulfuric acid less than is required to produce a collective float of both the lead and zinc sulfids, so as to form a froth in which the lead sulfid predominates, and thereafter submitting the tailings to a further froth flotation treatment with the addition of a frothing agent for the flotation of a froth in which the zinc sulfid predominates, and separating the froth.

In testimony whereof we have signed our names to this specification in the presence of two subscribing witnesses.

JAMES HEBBARD.  
RASMUS JOHN HARVEY.

Witnesses to the signature of James Hebbard:

ERNEST WILLIAM MOSS,  
GEORGE GUY TALMONDTH.

Witnesses to signature of Rasmus John Harvey:

ARTHUR GORE COLLISON,  
LESLIE HERBERT BROADBURY.